

## UNITED STATES PATENT OFFICE

2,059,304

METHOD OF COLD ROLLING COATED  
SHEET METAL

Lewis W. Beale and Joseph E. Murphy, Vandergrift, Pa., assignors to American Sheet and Tin Plate Company, a corporation of New Jersey

No Drawing. Application January 29, 1935,  
Serial No. 3,996

## 2 Claims. (CL. 80—60)

This invention pertains to a method of processing coated sheet metals. More particularly it relates to the processing of terne sheet or plate following the coating of the base metal with a lead-tin or "terne" mixture.

Terne sheet or plate originally was intended only as a roofing material which usually, in light gages and small sizes, is known as short terne. However, in recent years, heavy gage and large size sheet and plate have been terne coated and subjected to deep drawing operations resulting in gasoline tanks, automobile oil pans, caskets, etc., wherein the drawing characteristics of the base metal are aided by the terne coating which acts as a partial lubricant during the drawing operation. This grade, gage and size of sheet or plate is known as long terne, to distinguish it from the short terne coated roofing material.

In addition to the need for uniform drawability there have been imposed severe surface requirements upon long terne which have been difficult to meet due partially to the soft nature of this lead-tin coating.

Demands for smoothness of surface, flatness and proper behavior upon forming or drawing, together with the difficulty of cold rolling or roller leveling long terne sheets after they have been coated, have heretofore caused such cold rolling and roller leveling operations to be performed prior to the coating operation.

However, due to the phenomena of "aging" characteristic of iron and steel products as intensified by the heat of the pot in the coating operation, the coated sheets upon subsequent forming and/or bending show a tendency to give irregularly and locally which produces objectionable characteristics called "fluting". If the same material is subjected to stamping or drawing (rather than bending or forming) the irregular flow of metal produces so-called "stretcher strains". This tendency of the terne-coated sheet-like metal to "flue" or "stretcher strain" is traceable to the internal straining of the crystalline structure of the base metal during the coating operation.

Very severe and repeated cold rolling or roller leveling operations prior to coating will stiffen the sheets to a point where the heating of the pot will not bring back the full tendency of the sheets to flute or stretcher strain, but such excessive work on the sheets prior to coating is costly, and it also injures the ductility of the sheets, thus rendering them less suited for difficult forming or drawing operations.

This fluting and straining could be reduced

somewhat by roller leveling after coating, providing that the sheets were formed or stamped shortly thereafter for otherwise with time the effects of such roller leveling are soon lost.

A more substantial remedy for this tendency of the coated sheets to flute and stretcher strain is to cold roll such sheets after coating. If the proper amount of elongation is imposed on such coated sheets by such cold rolling the tendency to flute and stretcher strain is completely eliminated and the tendency for this condition to return is greatly delayed as compared to the rapid return of such tendencies after a mere roller leveling operation.

However, the coated sheets upon being thus cold rolled would slip and slide about between the rolls (due to the slippery nature of the coating) as to twist, camber or bow the sheets and cause the terne coating to take on a streaky appearance. The soft, slippery coating was readily susceptible to marking by the rolls and any loose particles thereon pitted the sheet almost instantaneously. This was particularly true of the excess coating upon the rear end of the sheets so coated, commonly known as "list end". This "list end" metal would leave the sheets and stick to the rolls, thus badly marking all subsequent sheets.

The slippage of these coated sheets when cold rolled was further accentuated by the presence of palm oil which as part of the coating procedure was not entirely removed in the cleaning of the coated metal in a so-called "branning machine".

Thus it was practically impossible to cold roll terne coated sheets to eliminate the tendency toward fluting and stretcher straining without incurring prohibitive damage to the sheets.

One of the objects of our invention is a practical method of cold rolling terne coated sheet metal in such a manner as to eliminate all tendency toward fluting or stretcher straining.

Another object is a method of cold rolling terne coated sheet metal as to eliminate all tendencies of the metal to flute or stretcher strain together with the elimination of excessive cold rolling or roller leveling of the sheet metal prior to the coating operation heretofore necessary.

Still another object is a method of cold rolling terne coated sheet metal in such a manner as to leave the coated sheet with a uniform overall surface finish.

A further object is a method of cold rolling terne coated sheet metal with no slippage of the sheets between the rolls and to the exclusion of cambered edges, such cold rolling taking place

40

45

50

55

without the necessity for removing all traces of oil from the surfaces of the coated sheet.

The above and other objects become more apparent to those skilled in the art from the reading 5 of the following specification and claims.

In carrying out our invention the base metal is hot rolled to gage in any convenient manner, such as strip or sheet, and thereafter properly heat treated to produce the physical properties 10 desired for satisfactory stamping, pressing or otherwise forming the metal in the manufacture of shaped articles.

After heat treating the base metal strip or sheet it is preferably processed to provide flatness 15 by providing a single cold roll pass or its equivalent as contrasted to the excessive cold working heretofore necessary.

The resulting sheet, after said cold rolled pass, has the desired ductility, surface and flatness and 20 the thus processed sheet is then preferably pickled, and then coated with a mixture of lead and tin to form terne sheets or plates in the usual manner. After the sheets are coated they are cleansed by passing through the usual branning machine, which removes the major and all 25 excess palm oil deposited during the terne coating operation. Those skilled in the art will readily recognize that some traces of palm oil remain on coated sheets after they have passed 30 through the branning machine, however, these traces of palm oil are not too detrimental to the processing of this invention, although they were detrimental in the processing methods of the prior art.

35 During the coating process, which is a hot process, there is a tendency to cause the base metal to stretcher strain or flute when worked such as by drawing or forming operations, and this tendency must be removed or eliminated in 40 order to provide satisfactory coated sheets for subsequent stamping, pressing or drawing. In order to remove the strains set up as a result of the coating process the coated sheets are cold rolled on a "wet" cold rolling mill. A "wet" mill, 45 which is well known in the art, comprises a set of rolls which are constantly flooded with a liquid, such as water, oil, or a combination of water and oil, so that the sheets passing through between said rolls are actually processed or rolled with 50 a film of water between each side of the sheet and the rolls. In other words, the pressure on the rolls is delivered to the sheets being processed through liquid films.

Heretofore attempts have been made to cold 55 roll terne coated sheets in dry cold rolling mills, however, the terne coated sheets had such a slippery surface as to make such rolling very difficult and in some cases almost impossible, and furthermore the slipping or moving of the sheets relative 60 to the roll when a dry mill is used marked and destroyed the surface of the sheets.

The art has long understood that "wet" mills 65 always have a lubricating effect and, recognizing the inherent slipperiness of terne coating, failed, as far as is known, to use the "wet" type of mill for cold rolling terne coated sheets in the belief that slippage would be aggravated.

We have discovered that by using a "wet" mill on terne coated sheets which have been cleaned only in the branning machine so that the sheets still retain traces of palm oil we can cold roll such terne coated sheets with excellent and im- 5 proved results.

We have discovered terne coated sheets rolled on a "wet" mill permits as great a reduction as is desired and necessary to remove the stretcher strains and fluting resulting from the heat of the 10 terne coating, with little or no pressure, and in extreme cases with an average maximum pressure necessary to result in a 2 per cent or 3 per cent elongation. The rolling under liquid produces a uniform surface finish of the terne coated sheets 15 which may vary from a bright surface resulting from the use of smooth rolls to a surface terne coat "silver frosting" resulting from the use of rough rolls. In the use of certain mills for this type of processing the rolls are usually turned as 20 truly cylindrical as possible and the blanket of liquid prevents dirt and dust from settling upon the rolls and the sheets being processed, thus resulting in a final sheet having an extremely smooth surface free from pits, dents, scratches 25 and the like. The extremely soft nature of the terne coating makes it extremely important to prevent the deposit of any foreign particles on the surface during the rolling operation or on the rolls with which the sheet is processed in order 30 to prevent the marring of the surface.

We have discovered further that by the use of a "wet" mill the liquid layer covering the rolls prevents any particles of excess metal on the "list" or "tail end" of the sheet from leaving the 35 sheet from adhering to the rolls, thus marring the surface of the sheet. Heretofore it has been difficult to prevent metal particles from leaving the sheet and adhering to the rolls of a dry cold rolling mill when rolling terne coated sheets. 40

We have also discovered that by the use of a "wet" mill, contrary to all expectations and teachings in the art, the terne coated sheets do not slip or slide in the mill and, therefore, marring 45 of the surfaces from this cause is prevented.

While we have described a certain specific embodiment of our invention it will be understood that we do not wish to be limited thereto, since various modifications may be made within the 50 scope of the appended claims.

We claim:

1. The method which includes rolling terne-coated sheets and plates in a cold wet mill whereby the slippage of the work-piece with respect to the mill rolls is reduced to a minimum. 55

2. The method which includes cold rolling a metallic sheet whereby inherent strains are established therein, terne-coating said cold rolled metallic sheet, subsequently rolling said terne-coated sheet in a cold mill to reduce the tendency of said sheet toward the development of said strains, and applying a liquid to the rolls of said cold mill to minimize slippage between said terne-coated sheet and said mill. 60

LEWIS W. BEALE.  
JOSEPH E. MURPHY.

65